

## UNITED STATES PATENT OFFICE

2,495,566

## PRODUCTION OF INSOLUBILIZED FILAMENTARY PRODUCTS BY THE WET SPINNING OF PROTEIN SOLUTIONS

Walter Anderson Caldwell, West Kilbride, and James Jack, Stevenston, Scotland, assignors to Imperial Chemical Industries Limited, a corporation of Great Britain

No Drawing. Application July 19, 1945, Serial No. 606,022. In Great Britain August 9, 1944

7 Claims. (Cl. 18—54)

1

The present invention relates to the manufacture of artificial filaments, threads, films or the like filamentary products obtained by the wet spinning of aqueous alkaline solutions of proteins, and especially of aqueous alkaline vegetable globulin and casein solutions, into saline aqueous coagulating baths of acid reaction and followed by a subsequent after-treatment of the filamentary products that includes a treatment with an insolubilising bath adapted to render the coagulated protein usefully resistant to treatment with boiling water, hot acid dyebaths and alkaline laundering solutions.

The filamentary products obtained by coagulation in the baths used for coagulating the extruded protein solutions require to be subjected to further chemical treatment to render them insoluble in water and resistant to the swelling or dissolving action of boiling water and weakly acidic and alkaline solutions, such as are used in dyeing and laundering. Such further chemical insolubilisation treatment is usually carried out with the aid of formaldehyde, chromium salts or aluminium salts, which are often referred to as hardening agents, in aqueous solutions containing such compounds in association with other solutes that increase their insolubilising action. Especially effective insolubilisation of the filamentary product may, for instance, be achieved by the method described in British Specification 513,910, which was accepted on October 25, 1939 and is an equivalent of U. S. Patent No. 2,347,677.

It is known that the stretching of the coagulated filament prior to its insolubilisation is beneficial to the strength of the resulting filamentary product.

It has been proposed to stretch the still acid coagulated filaments in a saline bath sufficiently hot to make them plastic, but when a bundle of parallel filaments is stretched in this manner they tend to stick together irreversibly when they are first wound up. When the saline bath is at a lower temperature this defect is not evidenced, but the amount of stretch that can be applied without breaking the filaments is less, and the stretched filaments are highly contractile.

The chemical insolubilisation treatment necessitates, for its progress to such a stage that the products become capable of drying without sticking together, a much longer time than is conven-

2

ient to apply to a continuously moving filamentary product. Accordingly it is desirable that for at least a considerable part of the period taken up by the insolubilisation treatment the filamentary product should be in an untensioned condition and that most of the insolubilisation treatment should take place after the tension employed in the coagulation step or in any subsequent stretching step, has been relaxed. While various treatments for the coagulated filamentary product intended to permit its insolubilisation to be effected in the untensioned condition have been proposed, they have been more or less unsatisfactory since the treatments have either taken an excessively long time so that they cannot conveniently be applied to the advancing filamentary product, and usually they have not enabled desirable extension of the filamentary product to be maintained when the tension is relaxed. The most rapid and satisfactory treatment has been to maintain the coagulated filament under tension in substantially saturated sodium chloride solution, for instance, as described in British Specification 543,586, which was accepted on March 4, 1942 and is an equivalent of U. S. Patent No. 2,358,427. When such treatment is carried out for about 10 minutes the tendency to longitudinal contraction of the filamentary material is thereby greatly reduced, and the subsequent insolubilisation step can be carried out on the relaxed filamentary material, for instance, in hank or staple form.

We have now found that desirably high permanent extension of the coagulated filamentary product, with corresponding advantage to the physical properties of the subsequently insolubilised product, can be attained if the coagulated, and if desired already somewhat stretched, filamentary product is stretched in an aqueous bath capable of swelling the filament and containing a solute adapted to buffer the fibre to a pH approximately the iso-electric point of the protein from which it is derived, and then washing the stretched filament without relaxing the tension in an aqueous non-solvent bath adapted to shrink it.

According to the present invention, therefore, the method for the manufacture from alkaline vegetable globulins and casein solutions of artificial filaments, threads, films or the like fila-

filamentary products of the kind hereinbefore defined comprises stretching the coagulum, obtained by the wet spinning of said alkaline solutions into saline coagulating bath of acid reaction, in an aqueous medium capable of swelling the coagulum and at a temperature such that the swollen and stretched coagulum remains contractile, said aqueous medium containing a solute such that the aqueous medium around the coagulum will approximate the isoelectric pH of the protein of the coagulum whereby the said aqueous medium around said coagulum will be of the acidity least capable of dissolving said protein, washing the swollen and stretched coagulum without relaxing the tension in an aqueous non-solvent non-hardening bath adapted to shrink it, whereby it is rendered non-contractile, and treating the resulting wet coagulum without the application of tension in an aqueous saline insolubilising bath adapted to render the coagulum usefully resistant to treatment with boiling water, hot acid dye baths and alkaline laundering solutions.

The acidity of the coagulated filamentary material emerging from the acid saline coagulating bath is preferably reduced by drawing it through one or more aqueous non-solvent baths, for instance, neutral saline baths, before subjecting it to the action of the swelling bath containing the buffering solute.

The buffering solute may comprise a weak base or feebly alkaline salt of a strong base with a weak acid, and may also comprise feebly acidic salts or weak acids in addition if necessary. As examples of weak bases and feebly basic salts, may be mentioned aniline, ortho-toluidine, sodium acetate, sodium citrate, and di-sodium hydrogen phosphate. If necessary citric acid, acetic acid, phosphoric acid, boric acid or mono sodium dihydrogen phosphate may be included. It will be understood that the total electrolyte concentration of the bath must not be excessive in order that it should retain the capacity to swell the filament. The bath may be used at atmospheric or preferably at a somewhat raised temperature.

The subsequent shrinking bath may be, for instance, a concentrated solution of a neutral salt or an organic dehydrating agent such as alcohol in water or some other non-solvent solution of like osmotic pressure.

If desired a preliminary stretch may be given to the filamentary product before it is introduced into the swelling bath of buffering properties in which it is stretched, for instance, in the coagulating bath or some intermediate bath such as a neutral saline bath.

The process according to the present invention has the advantage that the shrinking treatment applied to the stretched filament still under tension does not necessitate nearly such a long time as the treatments hitherto proposed for application to stretch the filament in order to render it possible to complete their insolubilisation without tension. Hence it can be more conveniently carried out on an advancing filament. Moreover, it enables a higher stretch to be applied, without rendering the filaments sticky, than the hitherto known stretching processes.

#### Example 1

A solution containing 25% by weight of pea nut protein 1.3% caustic soda and with a viscosity of 200 poises is extruded at the rate of 40 c. c. per minute through a spinneret containing 500 holes

each .09 mm. in diameter into a coagulating bath of 20% sodium sulphate and 2% sulphuric acid in water at 28° C. The filaments thus formed are drawn off over a 16 cm. diameter godet wheel 5 rotating at 90 revolutions per minute and passed through a second bath of 20% sodium sulphate in water at 40° C. and are collected on a swift at a peripheral speed of 60 metres per minute. The filaments are thereby extended about one third 10 of their length. After being kept on the swift in the sodium sulphate bath for about 20 minutes they are removed from it and placed in saturated brine at 20° C. A length of the filament is then withdrawn from the brine and stretched to twice 15 its length in 0.4% solution of aniline in water at 50° C. over a period of one minute and the extended filament is then transferred to a saturated sodium chloride bath and held for one minute in the stretched condition in the bath, which 20 is at 40° C., by which time the tension may be relaxed. The pH of the filament in the aniline bath is about 4.5.

The filaments are then transferred to an insolubilisation bath containing 1½% formaldehyde and 2% hydrochloric acid in saturated sodium chloride brine at 38° C., and are allowed to remain in this bath for eighteen hours, by which time they are capable of withstanding treatment in a bath containing 0.1% sulphuric acid and 30 0.25% sodium sulphate for 90 minutes at 97° C. The length of the filaments is 65% greater than that of the filaments taken from the swift, and the diameter of the filaments is correspondingly reduced. The iso-electric pH of pea nut protein 35 is about 4.5.

#### Example 2

In this case the coagulating bath is the same as in Example 1 and the freshly coagulated filaments as they are advanced are given a preliminary stretch in a bath of 20% sodium sulphate in water at 40° C. as in Example 1, but instead of being collected on a swift they are introduced from the tensioning roller into a bath consisting of 0.4% aniline solution in water at 50° C., in which they are further stretched to twice their length, and from this stretching bath the filaments pass over a series of successive pairs of skew cylindrical rollers driven to rotate at the same peripheral speed in parallel planes, over which they are wound in a helix so that they take one minute to complete the traverse. These skew rollers are immersed in saturated sodium chloride solution at 40° C., and thus hold the continuously advancing stretched filament at its stretched length in the saturated sodium chloride bath for one minute.

The advancing filaments are collected and cut into staple fibre. The staple fibre is then transferred to the insolubilisation bath described in Example 1, in which it is allowed to remain for eighteen hours at 30° C.

We claim:

1. In a method for the manufacture of artificial filamentary products of protein material by the wet-spinning of alkaline protein solutions into acidic saline coagulating baths, the steps which comprise stretching the coagulum in a weakly alkaline, non-hardening, swelling bath comprising an aqueous solution of an aryl amine at a temperature of between 20° C. and 50° C., washing the swollen and stretched coagulum without relaxing the tension with an aqueous, non-solvent, non-hardening, coagulum shrinking bath and 65 then insolubilizing the resulting product in un-

tensioned condition in an acidified concentrated saline formaldehyde bath.

2. The method as claimed in claim 1, wherein said coagulum shrinking bath is a concentrated solution of a neutral salt.

3. The method as claimed in claim 1, wherein the coagulum is subjected to a preliminary stretching operation in an aqueous, non-swelling bath prior to said stretching step in said weakly alkaline swelling bath.

4. The method as claimed in claim 1, wherein said coagulum shrinking bath is an aqueous solution of a water soluble alcohol.

5. In a method for the manufacture of artificial filamentary products of peanut protein material by the wet-spinning of alkaline peanut protein solutions into acidic saline coagulating baths, the steps which comprise stretching the coagulum in a weakly alkaline, non-hardening, swelling bath comprising an aqueous solution of an aryl amine at a temperature between 20° and 50° C., washing the swollen and stretched coagulum without relaxing the tension with a concentrated aqueous solution of a neutral salt and then insolubilizing

the resulting product in untensioned condition in an acidified concentrated saline formaldehyde bath.

6. The method as claimed in claim 5, wherein said aryl amine is aniline.

7. The method as claimed in claim 5, wherein said neutral salt solution is a saturated solution of sodium chloride.

WALTER ANDERSON CALDWELL.

JAMES JACK.

#### REFERENCES CITED

The following references are of record in the file of this patent:

#### UNITED STATES PATENTS

| Number    | Name     | Date          |
|-----------|----------|---------------|
| 2,211,961 | Meigo    | Aug. 20, 1940 |
| 2,266,672 | Wormell  | Dec. 16, 1941 |
| 2,290,789 | Wormell  | July 21, 1942 |
| 2,338,916 | Ferretti | Jan. 11, 1944 |
| 2,358,427 | Traill   | Aug. 19, 1944 |
| 2,409,475 | Cline    | Oct. 15, 1946 |